

## UNITED STATES PATENT OFFICE.

GORTON R. FONDA, OF SCHENECTADY, NEW YORK, ASSIGNOR TO GENERAL ELECTRIC COMPANY, A CORPORATION OF NEW YORK.

## INCANDESCENT FILAMENT.

No Drawing.

Application filed May 1, 1923. Serial No. 635,970.

The present invention relates to a novel refractory metal composition or alloy consisting largely of tungsten and containing thorium and copper as constituents, which is of particular utility as a lighting body in incandescent lamps. Filaments embodying my invention have a materially lower vapor pressure than an ordinary tungsten filament, and hence may be operated with a higher lighting efficiency than tungsten with the same average length of life, and if operated at the same efficiency will have a longer life. Although the production of my new incandescent material is not limited to any particular process, I find it convenient to employ in general the method of Coolidge U. S. Patent No. 1,082,933 of December 30, 1913. Thorium and copper may be added to tungsten in an elementary state, or as reducible or decomposable compounds. The following examples of tungsten compositions containing thorium and copper material will illustrate my invention.

To the finely divided metallic tungsten may be incorporated by weight 0.5% metallic thorium and 0.25% copper. This mixture is sintered and swaged as described in the above Coolidge patent whereby the material is rendered ductile. It is then drawn into filaments as described in this patent. The product when subjected to swaging and drawing has normally the small grain structure characteristic of thoriated tungsten wire, as described in Coolidge Patent No. 1,082,933. The specific electrical resistance of the swaged metal is materially higher than the specific resistance of substantially pure metallic tungsten, thoriated or non-thoriated,—say, in the neighborhood of 10% higher. It is substantially as workable as tungsten. At a given temperature the rate of evaporation of tungsten containing thorium and copper is less than that of either substantially pure tungsten or tung-

sten containing thorium alone. Incandescent filaments made in accordance with my invention may be mounted in vacuum lamps or in lamps containing a filling of gas or vapor, as described in Langmuir Patent No. 1,180,159. When filaments embodying my invention are to be operated in gas-filled lamps potassium silicate preferably is added to the raw batch of filament mix, as described in Patent No. 1,410,499, granted to Aladar Pacz, March 21, 1922.

What I claim as new and desire to secure by Letters Patent of the United States, is:

1. A composition consisting of tungsten in preponderating amount and containing fractional percentages of thorium and copper.

2. A sintered metal composition consisting in preponderating amount of tungsten and containing by weight about 0.50% thorium and 0.25% copper.

3. A filamentary body consisting largely of tungsten and containing associated therewith thorium and copper, said filament having at a given temperature of incandescence a rate of evaporation materially lower than substantially pure tungsten.

4. An incandescent lighting body operable at incandescence which consists in preponderating amount of tungsten and contains thorium and copper in combined amount of less than one per cent.

5. A metal composition consisting of a preponderating amount of tungsten and containing sufficiently large amounts of thorium and copper to cause the electrical resistance to be increased and the rate of evaporation at a given high temperature to be decreased as compared with tungsten unassociated with said materials.

In witness whereof, I have hereunto set my hand this 30th day of April, 1923.

GORTON R. FONDA.